# EUROPEAN PATENT SPECIFICATION

(11) **EP 2 785 900 B1**
(45) Date of publication and mention of the grant of the patent: **04.11.2015**
(21) Application number: 12791366.3
(22) Date of filing: 07.11.2012
(51) Int. Cl.: D01F 1/10, D01F 6/60, A46D 1/00, B08B 1/00, D01D 1/06

(54) **ABRASIVE FILAMENTS WITH IMPROVED STIFFNESS AND INDUSTRIAL BRUSHES COMPRISING THE SAME AND USES THEREOF**
SCHLEIFMITTELFILAMENTE MIT VERBESSERTER STEIFIGKEIT, INDUSTRIELLE BÜRSTEN DAMIT UND VERWENDUNGEN DAVON
FILAMENTS ABRASIFS PRÉSENTANT UNE RIGIDITÉ AMÉLIORÉE ET BROSSES INDUSTRIELLES LES COMPRENANT ET LEURS UTILISATIONS

(30) Priority: 29.11.2011 CN 201110386805
(43) Date of publication of application: 08.10.2014
(73) Proprietor: E. I. du Pont de Nemours and Company, Wilmington, DE 19898 (US); Dupont Xingda Filaments Company Limited, Huishan Distr., Wuxi Jiangsu 214183 (CN)
(72) Inventor: LIU, Xianqiao, Shanghai 201203 (CN); YU, Haifeng, Jiangsu 225002 (CN)
(74) Representative: Morf, Jan Stefan
(86) International application number: PCT/US2012/063984
(87) International publication number: WO 2013/081790

(56) References cited:
- WO-A1-2010/033671
- CN-A- 101 994 167
- DE-A1- 10 042 176
- JP-A- 5 279 916

## Description

### FIELD OF DISCLOSURE

The present disclosure is related to abrasive filaments with improved stiffness, industrial brushes comprising the abrasive filaments, and the uses of the industrial brushes.

### BACKGROUND

Abrasive filaments made from polyamides filled with abrasive particles were developed in the late 1950's as a man made alternative to natural abrasive filaments. At about that time an extrusion process was developed for dispersing abrasive particles uniformly in a polyamide matrix in the form of a filament (U.S. Patent Nos. 3,522,342 and 3,947,169). Some of the advantages of polyamide abrasive filaments are their safety, cleanliness, cutting speed, low cost, superior radius and finish control, adaptability, and ease to design.

A solar cell (also called photovoltaic cell or photoelectric cell) is a solid state electrical device that converts the energy of light directly into electricity by the photovoltaic effect. In crystal silicon based solar cells, silicon wafers are made by wire-sawing block-cast silicon ingots into very thin (180 to 350 µm) slices or wafers. A typical process of manufacturing silicon wafers often includes pulling a crystal silicon ingot; grinding the ingot; sawing off the ingot ends; and sawing up the ingot into wafers. In certain processes, the ingot is further polished using industrial brushes after the ingot ends are sawn off. Currently, polyamide based industrial brushes are often used in polishing the ingot. However, it is found that the polyamide based industrial brushes, due to the relative softness of the filaments, often causes end-rounding at the two longitudinal ends of the ingot and therefore reduces the production rate of silicon wafers. Thus, there is still a need to develop polyamide based abrasive filaments with improved stiffness and therefore increase the production rate of silicon wafers.

Various chain extending additives have been used in the prior art to improve the relative viscosity (RV) and other properties of polyamides. For example, U.S. Patent No. 7,005,097 discloses a polyamide composition in forming medical devices such as catheters or balloons. It is also disclosed that the addition of the bis-lactam compound, bis-oxazoline compound, or bis-oxazine compound based chain extending additive in the polyamide composition improves the RV of the composition and the wall strength of the medical device made therefrom. Further, PCT Patent Application No. WO2010033671 discloses the use of polycarbodiimide in polyamide based brush filaments to improve the hydrolysis resistance thereof. Yet, none of these references teaches that the addition of linear chain extending compounds may improve the flexural modulus or stiffness of polyamides.

### SUMMARY

One of the purpose of the present disclosure is to provide an abrasive filament with improved stiffness, wherein the abrasive filament is formed of a melt blended polyamide composition, and wherein the polyamide composition comprises: (a) at least one polyamide; (b) 0.1-1 wt% of at least one linear chain extending compound having a molecular weight of 1000 Daltons or lower; (c) 0.1-1 wt% of at least one antioxidant; and (d) 10-40 wt% of abrasive particles, with the total wt% of all components in the composition totaling to 100 wt%.

In one embodiment of the abrasive filament, the at least one linear chain extending compound is selected from the group consisting of bis-lactam compounds, bis-oxazoline compounds, bis-oxazine compounds, and combinations of two or more thereof. In such embodiments, the bis-lactam compounds are selected from the group consisting of N,N'-isophthaloyl bis-caprolactam; N,N'-adipoyl bis-caprolactam; N,N'-terephthaloyl bis-laurolactam; N,N'-isophthaloyl bis-butyrolactam; carbonyl bis-caprolactam; and combinations of two or more thereof, and the bis-oxazoline compounds and bis-oxazine compounds are selected from the group consisting of 2,2'-bis(2-oxazoline); 2,2-bis(4-methyl-2-oxazoline); 2,2'-bis(4-phenyl-2-oxazoline); 2,2'-bis(4-hexyloxazoline); 2,2'-p-phenylene bis(2-oxazoline); 2,2'-m-phenylene bis(2-oxazoline); 2,2'-tetramethylene bis(4,4'-dimethyl-2-oxazoline); the corresponding oxazines; and combinations or two or more thereof. Or, the at least one linear chain extending compound is carbonyl bis-caprolactam.

In a further embodiment of the abrasive filament, the at least one linear chain extending compound is present in the polyamide composition at a level of 0.2-0.7 wt%, based on the total weight of the polyamide composition.

In a yet further embodiment of the abrasive filament, the at least one antioxidant is selected from sterically hindered phenols. Or, the at least one antioxidant is selected from the group consisting of pentaerythritol tetrakis (3-(3,5-di-tert-butyl-4-hydroxyphenyl)propionate; 3,3',3',5,5',5'-hexa-tert-butyl-α,α',α'-(mesitylene-2,4-,6-triyl)tri-p-cresol; N,N'-hexane-1,6-diylbis(3-(3,5-di-tert-butyl-4-hydroxyphenylpropionamide)); octadecyl-3-(3,5-di-tert.butyl-4-hydroxyphenyl)-propionate; and combinations of two or more thereof. Or, the at least one antioxidant is N,N'-hexane-1,6-diylbis(3-(3,5-di-tert-butyl-4-hydroxyphenylpropionamide)).

In a yet further embodiment of the abrasive filament, the at least one antioxidant is present in the polyamide composition at a level of 0.2-0.7 wt%, based on the total weight of the polyamide composition.

In a yet further embodiment of the abrasive filament, the abrasive particles are selected from the group consisting of organic abrasive particles, inorganic abrasive particles, and combinations thereof. Or, the abrasive particles are selected from the group consisting of particles based on aluminum oxides, alpha alumina, silicon carbides, titanium diborides, alumina zirconia, diamond, boron carbide, ceria, aluminum silicates, cubic boron nitride, garnet, silica, pumice, sand, emery, mica, corundum, quartz, and combinations of two or more thereof.

In a yet further embodiment of the abrasive filament, the at least one polyamide is selected from aliphatic polyamides.

In a yet further embodiment of the abrasive filament, the at least one polyamide is selected from the group consisting of polyamide 4,6; polyamide 6; polyamide 6,6; polyamide 6,10; polyamide 6,12; polyamide 6,13; polyamide 6,14; polyamide 6,15; polyamide 6,16; polyamide 9,10; polyamide 9,12; polyamide 9,13; polyamide 9,14; polyamide 9,15; polyamide 9,36; polyamide 10,10; polyamide 10,12; polyamide 10,13; polyamide 10,14; polyamide 11; polyamide 12; polyamide 12,10; polyamide 12,12; polyamide 12,13; polyamide 12,14; and combinations of two or more thereof, or the at least one aliphatic polyamide is selected from polyamide 6,10; polyamide 6,12; and combinations thereof.

In a yet further embodiment of the abrasive filament, the at least one polyamide has a relative viscosity of 2.3-5, or 2.3-4, or 2.3-3.5.

In a yet further embodiment of the abrasive filament, the at least one polyamide is present in the polyamide composition at a level of 60-90 wt%, or 60-80 wt%, or 60-75 wt%, based on the total weight of the polyamide composition.

In a yet further embodiment of the abrasive filament, the abrasive filament is prepared by a continuous melt spinning process, and wherein the process comprises: (i) blending the at least one polyamide, the at least one linear chain extender compound, and the at least one antioxidant into a mixture; (ii) passing the mixture through an extruder while the abrasive particles are added into the extruder through one or more side feeders; and (iii) melt spinning the composition that comes out of the extruder into filaments.

In a yet further embodiment of the abrasive filament, the abrasive filament is prepared by a two-step melt spinning process, and wherein the process comprises: (i) melt compounding the at least one polyamide, the at least one linear chain extender compound, and the at least one antioxidant into resin pellets; (ii) passing the resin pellets through an extruder while the abrasive particles are added into the extruder through one or more side feeders; and (iii) melt spinning the composition that comes out of the extruder into filaments.

A further purpose of the present disclosure is to provide an industrial brush comprising a plurality of the abrasive filaments described above.

A yet further purpose of the present disclosure is to provide the use of the industrial brush described above in grinding and/or polishing silicon ingots, stone, or metal parts.

A yet further purpose of the present disclosure is to provide the use of the industrial brush in grinding and/or polishing silicon ingots.

In accordance with the present disclosure, when a range is given with two particular end points, it is understood that the range includes any value that is within the two particular end points and any value that is equal to or about equal to any of the two end points

### DETAILED DESCRIPTION

Disclosed herein are abrasive filaments formed of a melt blended polyamide composition, wherein the polyamide composition comprises: (a) at least one polyamide; (b) about 0.1-1 wt% of at least one linear chain extending compound having a molecular weight of about 1000 Daltons or lower; (c) about 0.1-1 wt% of at least one antioxidant, and (d) about 10-40 wt% of abrasive particles, with the total wt% of all components in the composition totaling to 100 wt%.

Polyamides are condensation copolymers formed by reacting equal parts of one or more diamines and one ore more dicarboxylic acids, so that amides are formed at both ends of each monomer in a process analogous to polypeptide biopolymers. It is understood that the polyamides used herein also include co-polyamides, which are copolymers formed by polymerizing two or more polyamide monomers or by reacting equal parts of two or more diamines and two or more dicarboxylic acids. In addition, the at least one polyamide comprised in the melt blended polyamide composition also may be a blend of two or more polyamides. Moreover, the polyamides used herein may have a relative viscosity (RV) of about 2.3-5, or about 2.3-4, or about 2.3-3.5.

Preferably, the polyamides used herein are aliphatic polyamides. The term "aliphatic polyamide" is used to refer to a polyamide containing no aromatic ring in its molecular chain and is a condensation product of an aminocarboxylic acid, a lactam, or a diamine and a dicarboxylic acid.

The aminocarboxylic acids used here may be aminocarboxylic acids having 6 to 12 carbon atoms, which include, but are not limited to, 6-aminocapronic acid, 7-aminoheptanoic acid, 9-aminononanoic acid, 11-aminoundecanoic acid, 12-aminododecanoic acid, and the like.
The lactam used here may be lactams having 4 to 12 carbon atoms, which include, but are not limited to, α-pyrrolidone, ε-caprolactam, ω-laurolactam, ε-enantholactam, and the like.

The diamines used here may be aliphatic or alicyclic diamines, including but not limited to, tetramethylenediamine; hexamethylenediamine; 2 methytpentamethylenediamine; nonamethylenediamine; undecamethylenediamine; dodeca-methylenediamine; 2,2,4-trimethylhexamethylenediamine; 2,4,4-trimethylhexamethylenediamine; 5-methylnonamethylene-diamine; 1,3-bis(aminomethyl)cyclohexane; 1,4-bis(aminomethyl)cyclohexane; 1-amino-3 aminomethyl-3,5,5-trimethylcyclohexane; bis(4-aminocyclohexyl)methane; bis(3-methyl-4-aminocyclohexyl)methane; 2,2-bis(4-aminocyclohexyl)propane; bis(aminopropyl)piperazine; aminoethylpiperazine; bis(p-aminocyclohexyl)methane; 2-methyloctamethylenediamine; trimethylhexamethylenediamine; 1,8-diaminooctane; 1,9-diaminononane; 1,10-diaminodecane; 1,12-diaminododecane; m-xylylenediamine; and the like.

The dicarboxylic acids used herein may be aliphatic or alicyclic dicarboxylic acids, including but riot limited to, adipic acid; glutaric acid; pimelic acid; suberic acid; azelaic acid; sebacic acid; dodecanedioic acid; 1,4-cyclohexanedicarboxylic acid; and the like.

Examples of preferred aliphatic polyamides include, but are not limited to, polyamide 4,6; polyamide 6; polyamide 6,6; polyamide 6,10; polyamide 6,12; polyamide 6,13; polyamide 6,14; polyamide 6,15; polyamide 6,16; polyamide 9,10; polyamide 9,12; polyamide 9,13; polyamide 9,14; polyamide 9,15; polyamide 9,36; polyamide 10,10; polyamide 10,12; polyamide 10,13; polyamide 10,14; polyamide 11; polyamide 12; polyamide 12,10; polyamide 12,12; polyamide 12,13; polyamide 12,14; and combinations of two or more thereof. In one embodiment, the at least one aliphatic polyamide comprised in the polyamide resin is selected from polyamide 6,10 ; polyamide 6,12; and combinations thereof.

In accordance to the present disclosure, the at least one polyamide may be present in the composition at a level of about 60-90 wt%, or about 60-80 wt%, or about 60-75 wt%.

The linear chain extending compounds used herein are low molecular weight (≤1000 Daltons) compounds that have bi-functional end groups. Such linear chain extending compounds are reactive with the terminal groups of polyamides but are essentially non-crosslinking. The at least one linear chain extending compound used herein may be selected from bis-lactam compounds, bis-oxazoline compounds, bis-oxazine compounds, and combinations of two or more thereof.

The bis-lactam compounds used herein may be represented by the following general formula (I): in which one or more of the methylene hydrogen atoms may alternatively be substituted by an alkyl or aryl radical; R represents a divalent organic radical; and n is an integer of 2-15.

In one embodiment, the R group in formula (I) may have a general formula (II): wherein A is a divalent organic group. Suitably A is a hydrocarbon group of about 20 carbons or less or a (poly)ether group. Exemplary A groups include, without limitation, alkylene groups (e.g., methylene; ethylene; 1,2 propylene; 1,3 propylene; or hexamethylene); arylene groups (e.g., phenylene; methylphenylene; naphthylene; 4,4'-biphenylene; a bisphenol A residue; or a bisphenol S residue); alkarylene groups (e.g., ethylenephenylene); and ether interrupted hydrocarbon groups (e.g., ethyleneoxyethylene; (polyethyleneoxy)ethylene; (polyethyleneoxy)propylene; or (polypropyleneoxy)ethylene).

In a further embodiment, the R group in formula (I) may have a general formula (III): wherein B is -NH-A-NH, with A being as previously defined.

In a yet further embodiment, the R group in formula (I) may simply be a carbonyl group with a general formula (IV): Compounds employing such carbonyl linkages are designated as "carbonyl bis-lactams". Suitable carbonyl bis-lactam compounds may have the general formula (V): in which n is an integer of 3-15, or preferably an integer of 5-12.

Bis-lactam compounds useful herein include those disclosed in U.S. Patent No. 6,228,980; PCT Patent Application No. WO 96/34909; and European Patent No. EP 0288253. Specific examples include, without limitation, N,N'-isophthaloyl bis-caprolactam; N,N'-adipoyl bis-caprolactam; N,N'-terephthaloyl bis-laurolactam; N,N'-isophthaloyl bis-butyrolactam; carbonyl bis-caprolactam; and combinations of two or more thereof.

The bis-oxazoline and bis-oxazine compounds used herein are both described by the formula (VI): where X is a divalent hydrocarbon group and the ring is a 5-membered ring for the bis-oxazoline or a 6-membered ring for the bis-oxazine, respectively; n=0 or 1; and D is a divalent organic group. And X may be an ethylene group, a substituted ethylene group, a trimethylene, or a substituted trimethylene group. As substituent, for instance an alkyl group with 1 to 10 carbon atoms, an aryl group, a cycloalkyl group, or an aralkyl group may be present. Exemplary alkyl groups include, without limitation, methyl, ethyl, hexyl, alkylhexyl, and nonyl groups; exemplary aryl groups include, without limitation, phenyl, naphthyl, and diphenyl groups; and exemplary cycloalkyl groups include, without limitation, cyclohexyl. D may be suitably a hydrocarbon group, e.g., an alkylene group, an arylene group, a cycloalkylene group, or an aralkylene group.

Examples of bis-oxazolines and bis-oxazines include, without limitation, 2,2'-bis(2-oxazoline); 2,2-bis(4-methyl-2-oxazoline); 2,2'-bis(4-phenyl-2-oxazoline); 2,2'-bis(4-hexyloxazoline); 2,2'-p-phenylene bis(2-oxazoline); 2,2'-p-phenylene bis(2-oxazoline); 2,2'-tetramethylene bis(4,4'-dimethyl-2-oxazoline); and the corresponding oxazines. Preference is given to 2,2'-bis(2-oxazoline); 2,2'-p-phenylene bis(2-oxazoline) (1,4-PBO); 2,2'-m-phenylene bis(2-oxazoline) (1,3-PBO); and the corresponding oxazines.

The linear chain extending compounds used herein also may be obtained commercially from various venders, which include, without limitation, carbonyl biscaprolactam (CBC) available from DSM (the Netherlands) under trade name ALLINCO^{™}; 1,4-phenylene bisoxazoline (1,4-PBO) available from DSM under trade name ALLINCO^{™}; and 2,2'-m-phenylene bis(2-oxazoline) (1,3-PBO) available from Takeda Chemical Industries (Japan) or from Mikuni Pharmaceutical Industrial Co., LTD. (Japan).

In accordance to the present disclosure, the at least one linear chain extending compound may be present in the polyamide composition at a level of about 0.1-1 wt% or about 0.2-0.7 wt%.

The process of incorporating the linear chain extending compounds can be carried out in a simple manner using the usual extruder melt-mixing techniques and equipment, for example by blending the terminally reactive polymer and the chain extender in a solid state. In some cases a small quantity (preferably no more than about 0.2%) of an oily processing aid may be added to the dry mix to improve the uniformity of distribution of the chain extender in the dry mix. The dry mix so obtained, is then melted in a conventional melt-mixing apparatus, for example a single- or double-screw extruder. Alternatively the polymer composition may be prepared in another type of melt mixer and then subsequently provided to the extruder directly from the initial melt mixer. The different components can also be fed to the extruder or other mixing apparatus separately. Chain extenders, in any form, can be fed into an extruder separately from the polymer resin by continuous feeding equipments.

Any suitable type of antioxidants may be used herein. Preferably, the antioxidants used herein are sterically hindered phenols. For examples, the antioxidants used herein may be selected from pentaerythritol tetrakis (3-(3,5-di-tert-butyl-4-hydroxyphenyl)propionate (CAS No. 6683-19-8, available from BASF (Germany) under the trade name Irganox^{™} 1010); 3,3',3',5,5',5'-hexa-tert-butyl-α,α',α'-(mesitylene-2,4-,6-triyl)trip-cresol (CAS No. 1709-70-2, available from BASF under the trade name Irganox^{™} 1330); N,N'-hexane-1,6-diylbis(3-(3,5-di-tert-butyl-4-hydroxyphenylpropionamide)) (CAS No. 23128-74-7, available from BASF under the trade name Irganox^{™} 1098); octadecyl-3-(3,5-di-tert.butyl-4-hydroxyphenyl)-propionate (CAS No. 2082-79-3, available from BASF under the trade name Irganox^{™} 1076); and combinations of two or more thereof.

In accordance to the present disclosure, the at least one antioxidant may be present in the polyamide composition at a level of about 0.1-1 wt% or about 0.2-0.7 wt%.

The abrasive particles used herein may be organic or inorganic and may have a particle size of about 0.1-1500 µm, or about 1-1000 µm, or about 50-500 µm.

Exemplary inorganic abrasive particles that are useful herein include, without limitation, aluminum oxides (e.g., fused aluminum oxides or heat treated aluminum oxides), alpha alumina, silicon carbides, titanium diborides, alumina zirconia, diamond, boron carbide, ceria, aluminum silicates, cubic boron nitride, garnet, silica, pumice, sand, emery, mica, corundum, quartz, and combinations of two or more thereof. Exemplary fused aluminum oxide particles include those available commercially from Exolon ESK Company (U.S.A.) or Washington Mills Electro Minerals Corp. (U.S.A.). Suitable ceramic aluminum oxide particles include those described in U.S. Patent Nos. 4,314,827; 4,623,364; 4,744,802; 4,770,671; 4,881,951; 4,964,883; 5,011,508; and 5,164,348. Suitable alpha alumina-based ceramic particles that comprise alpha alumina and rare earth oxide include those commercially available from 3M Company (U.S.A.) under the trade name CUBITRON^{™} 321. Also suitable herein are shaped abrasive particles, such as those disclosed in U.S. Patent Nos. 5,009,676; 5,185,012; 5,244,477; and 5,372,620. Other examples of particles useful herein include solid glass spheres, hollow glass spheres, calcium carbonate, polymeric bubbles, silicates, aluminum trihydirate, and mullite.

As used herein, the term abrasive particle also encompasses single abrasive particles which are bonded together to form an abrasive agglomerate. Abrasive agglomerates are further described in U.S. Patent Nos. 4,311,489; 4,652,275; and 4,799,939. The abrasive particles used herein may also contain a surface coating. Surface coatings are known to improve the adhesion between the abrasive particles and the binder. Suitable surface coatings are described in, e.g., U.S. Patent Nos. 5,011,508; 1,910,444; 3,041,156; 5,009,675; 4,997,461; 5,213,591; and 5,042,991. In some instances, the addition of the coating improves the abrading and/or processing characteristics of the abrasive particles.

Organic abrasive particles useful herein include those formed from a thermoplastic polymer and/or a thermosetting polymer. Organic abrasive particles useful herein may be individual particles or agglomerates of individual particles. The agglomerates may comprise a plurality of the organic abrasive particles bonded together by a binder to form a shaped mass.

The organic abrasive particles used herein may have any precise shape or may be irregularly or randomly shaped. Examples of such three dimensional shapes include, without limitation, pyramids, cylinders, cones, spheres, blocks, cubes, polygons, and the like. Alternatively, the organic abrasive particles may be relatively flat and have a cross sectional shape such as a diamond, cross, circle, triangle, rectangle, square, oval, octagon, pentagon, hexagon, polygon and the like.

The surface of the organic abrasive particles (a portion of their surface, or the entire surface) may be treated with coupling agents to enhance adhesion to and/or dispersibility in the molten thermoplastic matrix. The organic abrasive particles are not required to be uniformly dispersed in the hardened composition, but a uniform dispersion may provide more consistent abrasion characteristics.

The organic abrasive particles may be formed from a thermoplastic material such as polycarbonate, polyetherimide, polyester, polyvinyl chloride, methacrylate, methylmethacrylate, polyethylene, polysulfone, polystyrene, acrylonitrile-butadiene-styrene block copolymer, polypropylene, acetal polymers, polyurethanes, polyamide, and combinations thereof. In general, preferred thermoplastic material used herein as the organic abrasive particles are those having a high melting temperature, e.g. greater than 200°C or 300°C; or good heat resistance properties. Moreover, the organic abrasive particles need to have a higher melting or softening point than that of the thermoplastic matrix, so that the organic abrasive particles are not substantially affected by the filament manufacturing process. The organic abrasive particle should be capable of maintaining a generally particulate state during filament or brush segment processing, and therefore should be selected so as not to substantially melt or soften during the filament manufacturing process. In one preferred embodiment, the organic particles are selected to provide greater abrasive properties than the thermoplastic matrix, if present. In this manner, the organic abrasive particles will perform the desired surface refinement, such as removing foreign material from the workpiece or providing a fine surface finish, while the thermoplastic matrix wears away during operation to continuously present fresh organic abrasive particles to the workpiece surface.

There are several ways to form a thermoplastic abrasive particle. One such method is to extrude the thermoplastic polymer into elongate segments and then cut these segments into the desired length. Alternatively, the thermoplastic material can be molded into the desired shape and particle size. This molding process can be compression molding or injection molding.

The organic abrasive particles may be formed from a thermosetting polymer. Thermosetting polymers may be selected from phenolic resins, aminoplast resins, urethane resins, epoxy resins, acrylate resins, acrylated isocyanurate resins, ureaformaldehyde resins, isocyanurate resins, acrylated urethane resins, melamine formaldehyde resins, acrylated epoxy resins, and combinations of two or more thereof.

The organic abrasive particles used herein also may be formed from a mixture of a thermoplastic polymer and a thermosetting polymer.

Also in accordance to the present disclosure, the abrasive particles comprised in the composition may be a mixture of inorganic abrasive particles and organic particles.

In accordance to the present disclosure, the abrasive particles may be present in the composition at a level of about 10-40 wt%, or about 20-40 wt%, or about 25-40 wt%.

The abrasive filaments disclosed herein may be prepared by any suitable process, such as melt spinning processes. For example, the abrasive filaments may be prepared by a continuous melt spinning process, in which all components of the polyamide composition without the abrasive particles disclosed herein are blended together and then the blend is passed through an extruder (e.g., a twin-screw extruder) with the abrasive particles being added into the extruder through a side feeder and melt spun into filaments. Or, the abrasive filaments may be prepared by a two-step melt spinning process, in which all components of the polyamide composition without the abrasive particles are first melt compounded into resin pellets, and then the resin pellets are passed through an extruder (e.g., a twin-screw extruder), with the abrasive particles being added into the extruder through a side feeder, and melt spun into filaments.

As demonstrated by the examples below, before adding the abrasive particles, the base polyamide (e.g., polyamide 6,10) has a relatively low flexural modulus (e.g., 1548.8 MPa) (CE1). However, with the addition of the linear chain extending compound, along with the antioxidant, the flexural modulus of the base polyamide composition is greatly improved (an about 25% improvement, see E1). However, by adding branched chain extending additive (such as polycarbodiimide), the density of the base polyamide composition becomes too low to be processable and usable in practice (see CE2).

Further disclosed herein are industrial brushes comprising the abrasive filaments disclosed hereabove. The industrial brushes disclosed herein may be used for the grinding and/or polishing of silicon ingot, stone, or metal parts. In one embodiment, the industrial brushes disclosed herein are used for polishing silicon ingot. When used in polishing silicon ingots, industrial brushes comprising prior art abrasive filaments often cause severe end-rounding at the longitudinal end of the ingots and therefore decreases the production rate of silicon wafers. However, due to the improved flexural modulus or stiffness of the base polyamide composition that is used in the abrasive filaments disclosed herein, the end-rounding effect could be reduced and therefore the production rate of silicon wafers could be improved.

### EXAMPLES

### Material:

- PA610-1: a polyamide 6,10 having a relative viscosity (RV) of 2.73 and obtained from DuPont-Xingda Filaments Co. Ltd. (China) under trade name Herox^{®};
- PA610-2: a polyamide 6,10 having a RV of 2.35 and obtained from DuPont-Xingda Filaments Co. Ltd. (China) under trade name Herox^{®};
- PA612: a polyamide 6,12 having a RV of 2.5 and obtained from E.I. du Pont de Nemours and Company (U.S.A.) (hereafter "DuPont") under trade name Zytel^{®};
- AO: an antioxidant (N,N'-hexane-1,6-diylbis(3-(3,5-di-tert-butyl-4-hydroxyphenylpropionamide))) obtained from BASF (Germany) under trade name Irganox®1098;
- LCEC: a linear chain extending compound (N,N'-carbonyl biscaprolactam) obtained from DSM (Netherland) under the trade name ALLINCO^{™};
- BCEA: a branched chain extending additive (polycarbodiimide) obtained from Rhein Chemie (Germany) under the trade name Stabaxol^{™} P400;
- AP (abrasive particles): silicon carbide grits obtained from Jiangyan Dongyin Grinding Materials and Tools Co. Ltd. (China).

### Test Methods:

- RV (relative viscosity) was measured using ViscoSystem^{™} AVS 370 viscometer purchased from SI Analytics GmbH (Germany), wherein the test sampled were dissolved in a 98% sulfuric acid solution;
- MT (melt temperature) was measured using a Q100 Differential Scanning Calorimeter (DSC) (purchased from Texas Instruments (U.S.A.)) with the temperature ramp from 40°C to 280°C at a rate of 10°C/min;
- Tensile (tensile strength at break) was measured in accordance to ISO 527-2;
- EAB (elongation at break) was measured in accordance to ISO 527-2;
- FM (flexural modulus) was measured in accordance to ISO 178;
- Izod (Izod impact strength) was measured in accordance to ISO 180;
- Density was measured using an electronic densimeter SD-200L (purchased from Alfa Mirage Co. Ltd. (Japan)).

### Comparative Examples CE1-CE6 and Example E1:

All components contained in each of the polyamide compositions in Examples E1 and Comparative Examples CE1-CE6 and the amounts present are listed in Table 1 below. First, in each of CE2-E6 and E1, resin pellets comprising all components except abrasive particles were prepared by extrusion using a ZSK-30 twin-screw extruder (purchased from Coperion Werner & Pfleiderer GmbH & Co. (Germany)) with the extruder temperature set at 240-280°C, the extrusion speed at 300 rpm, and the throughput at 30 lb/hr. The RV for each of the resin pellets used in CE2-CE6 and E1 and the PA610-1 pellets used in CE1 were determined and the results are tabulated in Table 1. Thereafter, the resin pellets used in CE2-CE6 and E1 and the PA610-1 pellets used in CE1 were each molded into test specimens and the tensile strength at break, elongation at break, flexural modulus, and Izod impact strength thereof were determined and tabulated in Table 1. The test specimens used in these measurements were molded using a 180 ton injection molding machine purchased from Sumitomo Plastic Machinery (Japan) with a molding temperature set at about 250-260°C.

Finally, the resin pellets in each of CE1-CE6 and E1, along with 30 wt% of abrasive particles, were fed into a twin-screw extrusion spinning line to form filaments. The resin pellets were fed through the main feeder while the abrasive particles were fed through a side feed of the extruder and the extruder temperature was set at 240°-280°C. The density of the filaments were then determined and the results are tabulated in Table 1.

As it is shown here, before adding Abrasive Particles, PA610-1 has a relatively low flexural modulus (e.g., 1548.8 MPa) (CE1). However, with the addition of Linear Chain Extending Compound, along with Antioxidant, the flexural modulus of the base polyamide composition is greatly improved (an about 25% improvement, see E1). However, by adding Branched Chain Extending Additive, the density of the base polyamide composition becomes too low to be processable and usable in practice (see CE2).

**TABLE 1**

| | CE1 | CE2 | CE3 | CE4 | CE5 | CE6 | E1 |
|---|---|---|---|---|---|---|---|
| Composition | | | | | | | |
| PA610-1 (wt%) | 70 | 69.3 | 69.44 | 69.72 | 69.58 | 69.44 | 69.44 |
| AO (wt%) | - | - | 0.56 | 0.28 | - | - | 0.28 |
| LCEC (wt%) | - | - | - | - | 0.42 | 0.56 | 0.28 |
| BCEA (wt%) | - | 0.7 | - | - | - | - | - |
| AP (wt%) | 30 | 30 | 30 | 30 | 30 | 30 | 30 |

| Property | | | | | | | |
|---|---|---|---|---|---|---|---|
| RV | 2.73 | N/A | 2.95 | 3.02 | 3.14 | 3.19 | 3.08 |
| ¹MT (°C) | 219.8 | N/A | 221.1; | 221.1; | 221.3; | 221.4 | 221.8; |
| ¹Tensile (MPa) | 2006.2 | N/A | 2312 | 2291.2 | 2352.4 | 2352.1 | 2324.5 |
| ¹EAB (%) | 158.34 | N/A | 45.54 | 39.2 | 54.3 | 51.44 | 55.8 |
| ¹FM (MPa) | 1548.8 | N/A | 1830 | 1836.5 | 1920.3 | 1766.9 | 1937.6 |
| ¹Izod (KJ/m²) | 5.26 | N/A | 5.18 | 4.97 | 4.63 | 5.24 | 4.87 |
| Density (g/cm³) | 1.33 | 0.98 | 1.24 | 1.19 | 1.24 | 1.25 | 1.22 |

| | | | | | | | |
|---|---|---|---|---|---|---|---|
| Notes: ¹ The measurements of RV, MT, Tensile, EAB, FM, and Izod were obtained using the compositions without AP. | | | | | | | |

### Comparative Examples CE7-CE8 and Example E2-E4:

Similarly to E1 and CE2-CE6, the polyamide resin pellets used in E2-E4 and CE7-CE8 were prepared. The RV for each of the resin pellets used in E2-E4 and CE7-CE8 were determined and the results are tabulated in Table 2. Thereafter, the resin pellets used in E2-E4 and CE7-CE8 were molded into test specimens (as described above) and the tensile strength at break, elongation at break, flexural modulus, and Izod impact strength thereof were determined and tabulated in Table 2.

Again, as demonstrated herein, by adding Linear Chain Extending Compound and Antioxidant simultaneously into PA612, the flexural modulus therefore (E2) is improved compared to that of the PA612 compositions containing the Antioxidant (CE7) alone or that of the PA612 composition containing the Linear Chain Extending Compound alone (CE8).

**TABLE 2**

| | CE7 | CE8 | E2 | E3 | E4 |
|---|---|---|---|---|---|
| Composition | | | | | |
| PA612 (wt%) | 99.6 | 99.6 | 99.2 | 49.6 | - |
| AO (wt%) | 0.4 | - | 0.4 | 0.4 | 0.6 |
| LCEC (wt%) | - | 0.4 | 0.4 | 0.4 | 0.6 |
| PA610-2 (wt%) | - | - | - | 49.6 | 98.8 |

| Property | | | | | |
|---|---|---|---|---|---|
| RV | 2.69 | 2.86 | 2.79 | 2.63 | 2.51 |
| MT (°C) | 214.4 | 215.4 | 214.9 | 222.1 | 223.9 |
| Tensile (MPa) | 2209.5 | 2261.8 | 2200.5 | 1866.3 | 2081 |
| EAB (%) | 137.9 | 146.9 | 195.8 | 319.7 | 160.9 |
| FM (MPa) | 2131.0 | 2045.9 | 2151.2 | 1681.9 | 1911.4 |
| Izod (KJ/m²) | 5.47 | 5.43 | 5.50 | 6.29 | 5.59 |

## Claims

1. An abrasive filament formed of a melt blended polyamide composition, wherein the polyamide composition comprises:
(i) at least one polyamide;
(ii) 0.1-1 wt% of at least one linear chain extending compound having a molecular weight of 1000 Daltons or lower;
(iii) 0.1-1 wt% of at least one antioxidant; and
(iv) 10-40 wt% of abrasive particles,
with the total wt% of all components in the composition totaling to 100 wt%.

2. The abrasive filament of Claim 1, wherein the at least one linear chain extending compound is selected from the group consisting of bis-lactam compounds, bis-oxazoline compounds, bis-oxazine compounds, and combinations of two or more thereof, or preferably, the bis-lactam compounds are selected from the group consisting of N,N'-isophthaloyl bis-caprolactam; N,N'-adipoyl bis-caprolactam; N,N'-terephthaloyl bis-laurolactam; N,N'-isophthaloyl bis-butyrolactam; carbonyl bis-caprolactam; and combinations of two or more thereof, and the bis-oxazoline compounds and bis-oxazine compounds are selected from the group consisting of 2,2'-bis(2-oxazoline); 2,2-bis(4-methyl-2-oxazoline); 2,2'-bis(4-phenyl-2-oxazoline); 2,2'-bis(4-hexyloxazoline); 2,2'-p-phenylene bis(2-oxazoline); 2,2'-m-phenylene bis(2-oxazoline); 2,2'-tetramethylene bis(4,4'-dimethyl-2-oxazoline); the corresponding oxazines; and combinations of two or more thereof, or more preferably, the at least one linear chain extending compound is carbonyl bis-caprolactam.

3. The abrasive filament of Claim 1 or 2, wherein the at least one linear chain extending compound is present in the polyamide composition at a level of 0.2-0.7 wt%, based on the total weight of the polyamide composition.

4. The abrasive filament of any of Claims 1-3, wherein the at least one antioxidant is selected from sterically hindered phenols, or preferably, the at least one antioxidant is selected from the group consisting of pentaerythritol tetrakis (3-(3,5-di-tert-butyl-4-hydroxyphenyl)propionate; 3,3',3',5,5',5'-hexa-tert-butyl-α,α',α'-(mesitylene-2,4-,6-triyl)tri-p-cresol; N,N'-hexane-1,6-diylbis(3-(3,5-di-tert-butyl-4-hydroxyphenylpropionamide)); octadecyl-3-(3,5-di-tert.butyl-4-hydroxyphenyl)-propionate; and combinations of two or more thereof, or more preferably, the at least one antioxidant is N,N'-hexane-1,6-diylbis(3-(3,5-di-tert-butyl-4-hydroxyphenylpropionamide)).

5. The abrasive filament of any of Claims 1-4, wherein the at least one antioxidant is present in the polyamide composition at a level of 0.2-0.7 wt%, based on the total weight of the polyamide composition.

6. The abrasive filament of any of Claims 1-5, wherein the abrasive particles are selected from the group consisting of organic abrasive particles, inorganic abrasive particles, and combinations thereof, or preferably, the abrasive particles are selected from the group consisting of particles based on aluminum oxides, alpha alumina, silicon carbides, titanium diborides, alumina zirconia, diamond, boron carbide, ceria, aluminum silicates, cubic boron nitride, garnet, silica, pumice, sand, emery, mica, corundum, quartz, and combinations of two or more thereof.

7. The abrasive filament of any of Claims 1-6, wherein the at least one polyamide is selected from aliphatic polyamides, or preferably, the at least one polyamide is selected from the group consisting of polyamide 4,6; polyamide 6; polyamide 6,6; polyamide 6,10; polyamide 6,12; polyamide 6,13; polyamide 6,14; polyamide 6,15; polyamide 6,16; polyamide 9,10; polyamide 9,12; polyamide 9,13; polyamide 9,14; polyamide 9,15; polyamide 9,36; polyamide 10,10; polyamide 10,12; polyamide 10,13; polyamide 10,14; polyamide 11; polyamide 12; polyamide 12,10; polyamide 12,12; polyamide 12,13; polyamide 12,14; and combinations of two or more thereof, or more preferably, the at least one aliphatic polyamide is selected from polyamide 6,10; polyamide 6,12; and combinations thereof.

8. The abrasive filaments of any of Claims 1-7, wherein the at least one polyamide has a relative viscosity of 2.3-5, or preferably 2.3-4, or more preferably 2.3-3.5.

9. The abrasive filament of any of Claims 1-8, wherein the at least one polyamide is present in the polyamide composition at a level of 60-90 wt%, or preferably 60-80 wt%, or more preferably 60-75 wt%, based on the total weight of the polyamide composition.

10. The abrasive filament of any of Claims 1-9, wherein the abrasive filament is prepared by a continuous melt spinning process, and wherein the process comprises:
(i) blending the at least one polyamide, the at least one linear chain extender compound, and the at least one antioxidant into a mixture;
(ii) passing the mixture through an extruder while the abrasive particles are added into the extruder through one or more side feeders; and
(iii) melt spinning the composition that comes out of the extruder into filaments.

11. The abrasive filament of any of Claims 1-9, wherein the abrasive filament is prepared by a two-step melt spinning process, and wherein the process comprises:
(i) melt compounding the at least one polyamide, the at least one linear chain extender compound, and the at least one antioxidant into resin pellets;
(ii) passing the resin pellets through an extruder while the abrasive particles are added into the extruder through one or more side feeders; and
(iii) melt spinning the composition that comes out of the extruder into filaments.

12. An industrial brush comprising a plurality of the abrasive filaments of any of Claims 1-9.

13. The use of the industrial brush of Claim 12 in grinding and/or polishing silicon ingots, stone, or metal parts, or preferably the use in grinding and/or polishing silicon ingots.

## Patentansprüche

1. Schleifmittelfilament, das aus einer schmelzgemischten Polyamidzusammensetzung gebildet ist, wobei die Polyamidzusammensetzung Folgendes umfasst:
(i) mindestens ein Polyamid;
(ii) 0,1 - 1 Gew.-% mindestens einer linearen Kettenverlängerungsverbindung, die ein Molekulargewicht von 1000 Dalton oder weniger aufweist;
(iii) 0,1 - 1 Gew.-% mindestens eines Antioxidationsmittels; und
(iv) 10 - 40 Gew.-% Schleifmittelteilchen,
wobei die gesamten Gew.-% aller Komponenten in der Zusammensetzung sich insgesamt auf 100 Gew.-% belaufen.

2. Schleifmittelfilament nach Anspruch 1, wobei die mindestens eine lineare Kettenverlängerungsverbindung aus der Gruppe ausgewählt ist bestehend aus Bislactamverbindungen, Bisoxazolinverbindungen, Bisoxazinverbindungen und Kombinationen von zwei oder mehreren davon, oder bevorzugt die Bislactamverbindungen aus der Gruppe ausgewählt sind bestehend aus N,N'-Isophthaloylbiscaprolactam, N,N'-Adipoylbiscaprolactam, N,N'-Terephthaloylbislaurolactam, N,N'-Isophthaloylbisbutyrolactam, Carbonylbiscaprolactam und Kombinationen von zwei oder mehreren davon und die Bisoxazolinverbindungen und Bisoxazinverbindungen aus der Gruppe ausgewählt sind bestehend aus 2,2'-Bis(2-Oxazolin), 2,2-Bis(4-methyl-2-oxazolin), 2,2'-Bis(4-phenyl-2-oxazolin), 2,2'-Bis(4-hexyloxazolin, 2,2'-p-Phenylen-bis(2-oxazolin), 2,2'-m-Phenylen-bis(2-oxazolin), 2,2'-Tetramethylenbis-(4,4'-dimethyl-2-oxazolin), den entsprechenden Oxazinen und Kombinationen von zwei oder mehreren davon, oder noch bevorzugter die mindestens eine lineare Kettenverlängerungsverbindung Carbonylbiscaprolactam ist.

3. Schleifmittelfilament nach Anspruch 1 oder 2, wobei die mindestens eine lineare Kettenverlängerungsverbindung in der Polyamidzusammensetzung in einem Niveau von 0,2 - 0,7 Gew.-%, auf das Gesamtgewicht der Polyamidzusammensetzung bezogen, vorliegt.

4. Schleifmittelfilament nach einem der Ansprüche 1 - 3, wobei das mindestens eine Antioxidationsmittel aus sterisch gehinderten Phenolen ausgewählt ist oder bevorzugt das mindestens eine Antioxidationsmittel aus der Gruppe ausgewählt ist bestehend aus Pentaerythrittetrakis(3-(3,5-di-tert-butyl-4-hydroxyphenyl)propionat, 3,3',3',5,5',5'-Hexa-tert-butyl-α,α',α'-(mesitylen-2,4-,6-triyl)tri-p-cresol, N,N'-Hexan-1,6-diylbis(3-(3,5-di-tert-butyl-4-hydroxyphenyl)-propionat und Kombinationen von zwei oder mehreren davon oder noch bevorzugter das mindestens eine Antioxidationsmittel N,N'-Hexan-1,6-diylbis(3-(3,5-di-tert-butyl-4-hydroxyphenylpropionamid)) ist.

5. Schleifmittelfilament nach einem der Ansprüche 1 - 4, wobei das mindestens eine Antioxidationsmittel in der Polyamidzusammensetzung in einem Niveau von 0,2 - 0,7 Gew.-%, auf das Gesamtgewicht der Polyamidzusammensetzung bezogen, vorliegt.

6. Schleifmittelfilament nach einem der Ansprüche 1 - 5, wobei die Schleifmittelteilchen aus der Gruppe ausgewählt sind bestehend aus organischen Schleifmittelteilchen, anorganischen Schleifmittelteilchen und Kombinationen davon oder bevorzugt die Schleifmittelteilchen aus der Gruppe ausgewählt sind bestehend aus Teilchen auf der Basis von Aluminiumoxiden, Alpha-Aluminiumoxid, Siliciumcarbiden, Titandiboriden, Aluminiumoxid-Zirconiumdioxid, Diamant, Borcarbid, Ceroxid, Aluminiumsilicaten, kubischem Bornitrid, Granat, Siliciumdioxid, Bimsstein, Sand, Schmirgel, Glimmer, Korund, Quarz und Kombinationen von zwei oder mehreren davon.

7. Schleifmittelfilament nach einem der Ansprüche 1 - 6, wobei das mindestens eine Polyamid von aliphatischen Polyamiden ausgewählt ist oder bevorzugt das mindestens eine Polyamid aus der Gruppe ausgewählt ist bestehend aus Polyamid 4,6, Polyamid 6, Polyamid 6,6, Polyamid 6,10, Polyamid 6,12, Polyamid 6,13, Polyamid 6,14, Polyamid 6,15, Polyamid 6,16, Polyamid 9,10, Polyamid 9,12, Polyamid 9,13, Polyamid 9,14, Polyamid 9,15, Polyamid 9,36, Polyamid 10,10, Polyamid 10,12, Polyamid 10,13, Polyamid 10,14, Polyamid 11, Polyamid 12, Polyamid 12,10, Polyamid 12,12, Polyamid 12,13, Polyamid 12,14, und Kombinationen von zwei oder mehreren davon, oder noch bevorzugter das mindestens eine aliphatische Polyamid aus Polyamid 6,10, Polyamid 6,12 und Kombinationen davon ausgewählt ist.

8. Schleifmittelfilamente nach einem der Ansprüche 1 - 7, wobei das mindestens eine Polyamid eine relative Viskosität von 2,3 - 5, oder bevorzugt 2,3 - 4 oder noch bevorzugter 2,3 - 3,5 aufweist.

9. Schleifmittelfilament nach einem der Ansprüche 1 - 8, wobei das mindestens eine Polyamid in der Polyamidzusammensetzung in einem Niveau von 60 - 90 Gew.-% oder bevorzugt 60 - 80 Gew.-% oder noch bevorzugter 60 - 75 Gew.-%, auf das Gesamtgewicht der Polyamidzusammensetzung bezogen, vorliegt.

10. Schleifmittelfilament nach einem der Ansprüche 1 - 9, wobei das Schleifmittelfilament durch ein kontinuierliches Schmelzspinnverfahren hergestellt wird und wobei das Verfahren Folgendes umfasst:
(i) das Vermischen des mindestens einen Polyamids, der mindestens einen linearen Kettenverlängerungsverbindung und des mindestens einen Antioxidationsmittels zu einer Mischung;
(ii) das Hindurchführen der Mischung durch einen Extruder, während die Schleifmittelteilchen in den Extruder durch eine oder mehrere Seitenzuliefervorrichtungen eingegeben werden; und
(iii) das Schmelzspinnen der Zusammensetzung, die aus dem Extruder austritt, zu Filamenten.

11. Schleifmittelfilament nach einem der Ansprüche 1 - 9, wobei das Schleifmittelfilament durch ein Zweischritt-Schmelzspinnverfahren hergestellt wird und wobei das Verfahren Folgendes umfasst:
(i) das Schmelzcompoundieren des mindestens einen Polyamids, der mindestens einen linearem Kettenverlängerungsverbindung und des mindestens einen Antioxidationsmittels zu Harzkügelchen;
(ii) das Hindurchführen der Harzkügelchen durch einen Extruder, während die Schleifmittelteilchen durch eine oder mehrere Seitenzuliefervorrichtungen in den Extruder eingegeben werden; und
(iii) das Schmelzspinnen der Zusammensetzung, die aus dem Extruder austritt, zu Filamenten.

12. Industrielle Bürsten umfassend eine Mehrzahl der Schleifmittelfilamente nach einem der Ansprüche 1 - 9.

13. Verwendung der industriellen Bürste nach Anspruch 12 zum Schleifen und/oder Polieren von Siliciumbarren, Stein oder Metallteilen oder bevorzugt Verwendung zum Schleifen und/oder Polieren von Siliciumbarren.

## Revendications

1. Filament abrasif formé d'une composition de polyamide mélangée à l'état fondu, dans lequel la composition de polyamide comprend:
(i) au moins un polyamide;
(ii) 0,1 à 1% en poids d'au moins un composé allongeur de chaîne linéaire ayant un poids moléculaire de 1000 daltons ou moins;
(iii) 0,1 à 1% en poids d'au moins un antioxydant; et
(iv) 10 à 40% en poids de particules abrasives,
le % en poids total de tous les constituants dans la composition s'élevant à 100% en poids.

2. Filament abrasif selon la revendication 1, dans lequel ledit au moins un composé allongeur de chaîne linéaire est choisi dans le groupe constitué par les composés bis-lactames, les composés bis-oxazolines, les composés bis-oxazines, et des combinaisons de deux ou plus de ceux-ci, ou de préférence, les composés bis-lactames sont choisis dans le groupe constitué par le N,N'-isophtaloyl bis-caprolactame; le N,N'-adipoyl bis-caprolactame; le N,N'-téréphtaloyl bis-laurolactame; le N,N'-isophtaloyl bis-butyrolactame; le carbonyl bis-caprolactame; et des combinaisons de deux ou plus de ceux-ci, et les composés bis-oxazolines et les composés bis-oxazines sont choisis dans le groupe constitué par la 2,2'-bis(2-oxazoline); la 2,2-bis(4-méthyl-2-oxazoline); la 2,2'-bis(4-phényl-2-oxazoline); la 2,2'-bis(4-hexyloxazoline); la 2,2'-p-phénylène bis(2-oxazoline); la 2,2'-m-phénylène bis(2-oxazoline); la 2,2'-tétraméthylène bis(4,4'-diméthyl-2-oxazoline); les oxazines correspondantes; et des combinaisons de deux ou plus de celles-ci, ou de préférence encore, ledit au moins un composé allongeur de chaîne linéaire est le carbonyl bis-caprolactame.

3. Filament abrasif selon la revendication 1 ou 2, dans lequel ledit au moins un composé allongeur de chaîne linéaire est présent dans la composition de polyamide à un taux de 0,2 à 0,7% en poids, par rapport au poids total de la composition de polyamide.

4. Filament abrasif selon l'une quelconque des revendications 1 à 3, dans lequel ledit au moins un antioxydant est choisi parmi les phénols empêchés stériquement, ou de préférence, ledit au moins un antioxydant est choisi dans le groupe constitué par le tétrakis (3-(3,5-di-tert-butyl-4-hydroxyphényl)propionate de pentaérythritol; le 3,3',3',5,5',5'-hexa-tert-butyl-α,α',α'-(mésitylène-2,4-,6-triyl)tri-p-crésol; le N,N'-hexane-1,6-diylbis(3-(3,5-di-tert-butyl-4-hydroxyphénylpropionamide)); l'octadécyl-3-(3,5-di-tert.butyl-4-hydroxyphényl)-propionate; et des combinaisons de deux ou plus de ceux-ci, ou de préférence encore, ledit au moins un antioxydant est le N,N'-hexane-1,6-diylbis(3-(3,5-di-tert-butyl-4-hydroxyphénylpropionamide)).

5. Filament abrasif selon l'une quelconque des revendications 1 à 4, dans lequel ledit au moins un antioxydant est présent dans la composition de polyamide à un taux de 0,2 à 0,7% en poids, par rapport au poids total de la composition de polyamide.

6. Filament abrasif selon l'une quelconque des revendications 1 à 5, dans lequel les particules abrasives sont choisies dans le groupe constitué par les particules abrasives organiques, les particules abrasives inorganiques, et des combinaisons de celles-ci, ou de préférence, les particules abrasives sont choisies dans le groupe constitué par les particules à base d'oxydes d'aluminium, l'alpha alumine, les carbures de silicium, les diborures de titane, l'alumine et zircone, le diamant, le carbure de bore, l'oxyde de cérium, les silicates d'aluminium, le nitrure de bore cubique, le grenat, la silice, la pierre ponce, le sable, l'émeri, le mica, le corindon, le quartz, et des combinaisons de deux ou plus de ceux-ci.

7. Filament abrasif selon l'une quelconque des revendications 1 à 6, dans lequel ledit au moins un polyamide est choisi parmi les polyamides aliphatiques, ou de préférence, ledit au moins un polyamide est choisi dans le groupe constitué par le polyamide 4,6; le polyamide 6; le polyamide 6,6; le polyamide 6,10; le polyamide 6,12; le polyamide 6,13; le polyamide 6,14; le polyamide 6,15; le polyamide 6,16; le polyamide 9,10; le polyamide 9,12; le polyamide 9,13; le polyamide 9,14; le polyamide 9,15; le polyamide 9,36; le polyamide 10,10; le polyamide 10,12; le polyamide 10,13; le polyamide 10,14; le polyamide 11; le polyamide 12; le polyamide 12,10; le polyamide 12,12; le polyamide 12,13; le polyamide 12,14; et des combinaisons de deux ou plus de ceux-ci, ou de préférence encore, ledit au moins un polyamide aliphatique est choisi parmi le polyamide 6,10; le polyamide 6,12; et des combinaisons de ceux-ci.

8. Filaments abrasifs selon l'une quelconque des revendications 1 à 7, dans lesquels ledit au moins un polyamide a une viscosité relative de 2,3 à 5, ou de préférence 2,3 à 4 ou de préférence encore 2,3 à 3,5.

9. Filament abrasif selon l'une quelconque des revendications 1 à 8, dans lequel ledit au moins un polyamide est présent dans la composition de polyamide à un taux de 60 à 90% en poids, ou de préférence 60 à 80% en poids, ou de préférence encore 60 à 75% en poids, par rapport au poids total de la composition de polyamide.

10. Filament abrasif selon l'une quelconque des revendications 1 à 9, lequel filament abrasif est préparé par un procédé de filage par fusion continu, et dans lequel le procédé consiste:
(i) à mélanger ledit au moins un polyamide, ledit au moins un composé allongeur de chaîne linéaire et ledit au moins un antioxydant en un mélange;
(ii) à faire passer le mélange à travers une extrudeuse pendant que les particules abrasives sont ajoutées dans l'extrudeuse à travers un ou plusieurs dispositifs d'alimentation latéraux; et
(iii) à filer par fusion la composition qui sort de l'extrudeuse en filaments.

11. Filament abrasif selon l'une quelconque des revendications 1 à 9, lequel filament abrasif est préparé par un procédé de filage par fusion à deux étapes, et dans lequel le procédé consiste:
(i) à mélanger à l'état fondu ledit au moins un polyamide, ledit au moins un composé allongeur de chaîne linéaire et ledit au moins un antioxydant en granules de résine;
(ii) à faire passer les granules de résine à travers une extrudeuse pendant que les particules abrasives sont ajoutées dans l'extrudeuse à travers un ou plusieurs dispositifs d'alimentation latéraux; et
(iii) à filer par fusion la composition qui sort de l'extrudeuse en filaments.

12. Brosse industrielle comprenant une pluralité des filaments abrasifs selon l'une quelconque des revendications 1 à 9.

13. Utilisation de la brosse industrielle selon la revendication 12 dans le meulage et/ou le polissage de lingots de silicium, d'une pierre ou de pièces métalliques, ou de préférence utilisation dans le meulage et/ou le polissage de lingots de silicium.
